

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 1

Figure 1



Figure 2



Figure 3



Figure 4



INVENTOR:  
Edward Michalko

BY:

James R. Hooton Jr.  
Robert W. Erickson

ATTORNEYS

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 2

Figure 5



INVENTOR:  
Edward Michalko

BY: James R. Hoateon Jr.  
Robert W. Erickson  
ATTORNEYS

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 3

Figure 6



INVENTOR:  
Edward Michalko

BY:

James R. Houston Jr.  
Robert W. Erickson  
ATTORNEYS

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 4



Figure 7

INVENTOR:  
Edward Michalko

BY:  
James P. Hooton Jr.  
Robert W. Erickson

ATTORNEYS

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 6



Figure 8

INVENTOR:  
Edward Michalko  
BY: James P. Hartson Jr.  
Robert W. Erickson  
ATTORNEYS

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 6



Figure 9

INVENTOR:  
Edward Michalko

BY: *James R. Hasteen Jr.*  
*Robert W. Erickson*  
ATTORNEYS

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 7



Figure 10

INVENTOR:  
Edward Michalko

BY: *James R. Watson Jr.*  
*Robert W. Erickson*  
ATTORNEYS

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 8



Figure II

INVENTOR:  
Edward Michalko

BY: James P. Hutton Jr.  
Robert W. Erickson  
ATTORNEYS

July 5, 1966

E. MICHALKO

3,259,454

METHOD OF OXIDIZING GASEOUS COMBUSTIBLE WASTE PRODUCTS

Original Filed April 20, 1962

9 Sheets-Sheet 9



Figure 12

INVENTOR:  
Edward Michalko

BY: *James P. Hoatson Jr.*  
*Robert W. Erickson*  
ATTORNEYS

1

3,259,454

## METHOD OF OXIDIZING GASEOUS COMBUSTIBLE WASTE PRODUCTS

Edward Michalko, Chicago, Ill., assignor to Universal Oil Products Company, Des Plaines, Ill., a corporation of Delaware

Original application Apr. 20, 1962, Ser. No. 189,101.  
Divided and this application Aug. 26, 1963, Ser. No. 304,381

4 Claims. (Cl. 23—2)

This application is a division of my copending application, Serial Number 189,101, filed April 20, 1962, and is being filed to comply with a requirement for restriction of invention.

In a broad scope, the present invention relates to the treatment of combustible waste products, containing pollutants having noxious characteristics, prior to discharging the same into the atmosphere. The present invention involves the preparation of a catalytic composite having a novel physical structure heretofore not obtained, and the use of such catalytic composite. More specifically, the invention described herein is directed toward the use of a catalyst, having particular characteristics, in the conversion of gaseous, combustible waste products of a noxious nature, into innocuous components for the primary purpose of eliminating the adverse effects exhibited by such waste products upon the atmosphere.

The catalytic composite encompassed by the present invention is especially adaptable to the elimination of the products of incomplete combustion from the hydrocarbonaceous exhaust gases emanating from an internal combustion engine, prior to effecting the discharge of such hydrocarbonaceous exhaust gases into the atmosphere.

The desirability and importance of effecting the removal of noxious components from automotive exhaust gases, or the conversion thereof into innocuous components, has recently been recognized. The incomplete combustion of hydrocarbon fuels by the gasoline, or diesel engine results in the generation of substantial quantities of unburned hydrocarbons, and other undesirable products, which, while being of a noxious nature, discharge into the atmosphere through the exhaust line as gaseous waste material. With the ever-increasing concentration of automobiles, particularly in the more densely populated urban areas, the discharge of deleterious, noxious matter into the atmosphere rapidly attains significantly detrimental proportions. Under the influence of sunlight, it is believed that these undesirable products of incomplete combustion react with atmospheric oxygen to produce a dense, polluted atmosphere now commonly referred to as smog. Such undesirable hydrocarbonaceous combustion products include, for example, unsaturated hydrocarbons, particularly oxidized hydrocarbons such as alcohols, ketones, aldehydes, and acids, etc., carbon monoxide, and various oxides of nitrogen and sulfur. At least one State, California, has passed legislation recognizing the inherent danger to the public health and welfare as such noxious gaseous material continues to be discharged into the atmosphere, and, in this regard, has appropriately instituted a Motor Vehicle Pollution Control Board having as its primary purpose the elimination, or conversion of these noxious components.

The discharge of noxious products of incomplete combustion, emanating from internal combustion engines, is but one source of pollution of the atmosphere. Although described with particular reference to the catalytic

2

conversion, or elimination, of such noxious exhaust gases, the present invention will be found readily adaptable, by those skilled within the art, for utilization in conjunction with diesel engines, butane engines, natural gas engines, and the like. Other examples of the discharge of deleterious gaseous waste material into the atmosphere include the waste gases from stationary units such as large internal combustion engines for driving pumps, compressors and generators, waste-heat boilers, and flue-gas power recovery units, etc. The use of the present invention is advantageous in removing deleterious contaminating components from waste products characterized by the fumes exhausted from a variety of industrial operations including the printing industry, the tanning industry, and various heavy chemical industries. For example, in the printing industry, a variety of inks, dyes, and the like, contain hydrocarbons and other chemical compounds, which, either in the same or modified form, accumulate within the surroundings and are vented into the atmosphere by blowers, fans, etc. An example of the chemical process and industry, to which the present invention is suitably well adapted, is the process involved in the manufacture of phthalic anhydride. Thus, although particularly directed toward the conversion of a hydrocarbonaceous combustible mixture emanating from an internal combustion engine, the present invention affords a method for treating a variety of noxious, gaseous waste products for the purpose of decreasing the deleterious effect which is otherwise encountered by discharging such noxious waste products into the atmosphere.

The primary object of the present invention is, therefore, to provide a method for the catalytic treatment, and the catalyst for use therein, of noxious, combustible gaseous waste products for the purpose of eliminating the noxious material and/or converting the same into innocuous components. A related object is to produce a catalytic composite having a novel physical structure and the propensity for effecting the conversion of a hydrocarbon-containing mixture, as well as the capability to effect such conversion for a prolonged period of time.

A broad embodiment of the present invention encompasses a catalytic particle comprising an inorganic oxide carrier material and a catalytically active metallic component imbedded as a layer within said carrier material, and disposed a finite distance below the exterior surface of said carrier material and a finite distance from the center thereof.

Another broad embodiment of the present invention involves a method of preparing a catalytic composite which comprises commingling an inorganic oxide carrier material with a catalytically active metallic component and from about 0.1% to about 1.5% by weight, based upon the weight of said carrier material, of an organic acid selected from the group consisting of dibasic acids and derivatives thereof, having the following structural formula:



where:

R is selected from hydrogen, hydroxyl and alkyl groups;

R' is selected from hydrogen, alkyl and carboxyl groups;

and

n is within the range of 0 to 6.

A more specific embodiment of the present invention affords a method of preparing a catalytic composite of alumina and a platinum component, which method comprises commingling said alumina with chloroplatinic acid and from about 0.13% to about 0.70% by weight, based upon the weight of said alumina, of an organic acid selected from the group consisting of dibasic acids and derivatives thereof, having the following structural formula:



where:

R is selected from hydrogen, hydroxyl and alkyl groups; R' is selected from hydrogen, alkyl and carboxyl groups; and n is within the range of 0-6,

drying the resulting mixture at a temperature within the range of from about 100° F. to about 250° F., and thereafter subjecting the mixture to an atmosphere of hydrogen at a temperature within the range of from about 900° F. to 1800° F.

As hereinbefore stated, the present invention produces a catalytic composite especially adaptable for the conversion of noxious, combustible gaseous waste products into innocuous components, prior to discharging such waste products into the atmosphere. Therefore, another broad embodiment of the present invention relates to a method for the conversion of noxious, gaseous combustible waste products to be discharged into the atmosphere, which method comprises contacting said waste products with a catalytic composite of an inorganic oxide carrier material and a catalytically active metallic component imbedded as a layer within said carrier material, and disposed a finite distance below the exterior surface of said carrier material and a finite distance from the center thereof.

Another limited embodiment of the present invention involves a method for eliminating hydrocarbons from gases containing the same which comprises contacting said gases, at conversion conditions, with a catalytic composite of alumina and a platinum component, said catalytic composite being prepared by initially commingling said alumina with a platinum-containing compound and from about 0.13% to about 0.70% by weight, based upon the weight of said alumina, of an organic acid selected from the group consisting of dibasic acids and derivatives thereof, having the following structural formula:



where:

R is selected from hydrogen, hydroxyl and alkyl groups; R' is selected from hydrogen, alkyl and carboxyl groups; and n is within the range of 0-6.

The present invention particularly provides a method for eliminating products of incomplete combustion from the hydrocarbonaceous exhaust gases emanating from an internal combustion engine, which method comprises contacting said exhaust gases, at conversion conditions, with a catalytic composite of alumina and a platinum component imbedded as a layer within said alumina and disposed a finite distance below the exterior surface of said alumina and a finite distance from the center thereof; said catalytic composite having been prepared by initially commingling said alumina with a platinum-containing compound and from about 0.13% to about 0.70% by weight, based upon the weight of said alumina, of an

organic acid selected from the group consisting of dibasic acids and derivatives thereof, having the following structural formula:



where:

10 R is selected from hydrogen, hydroxyl and alkyl groups; R' is selected from hydrogen, alkyl and carboxyl groups; and n is within the range of 0-6.

15 As hereinbefore set forth, the method of the present invention involves the catalytic treatment of noxious, gaseous combustible waste products prior to discharging the same into the atmosphere. The catalytic composite for use therein, hereinafter described in detail, may be placed in any suitable container, or catalytic convertor, and installed within the exhaust line in such a manner that the gaseous waste products are passed therethrough. The catalytic convertor may be of the through-flow, cross-flow, or radial-flow design, and, when utilized in the 20 conversion of the noxious components emanating from an internal combustion engine, may either supplant, or be combined with the common acoustic muffler. Combustion air is injected ahead of the convertor inlet, usually by an aspirator or suitable external compressive means, and the waste products, together with air, are passed through the catalyst in either upward or downward flow, cross-flow or radial-flow. When employed in other applications, such as the treatment of the gaseous waste products from the printing, tanning and petrochemical industries, the catalytic composite may be conveniently disposed as a fixed-bed within the stack, or other outlet ducts, of a suitable combustion chamber, the combustion products and air being passed in admixture into contact with the catalyst prior to being discharged into the atmosphere. The precise physical structure of the catalytic 25 convertor, the means for introducing combustion air, and the disposition of the catalytic composite within the convertor are dependent to a large extent upon the application and the function to be served.

30 45 A wide variety of factors affect the stability of active catalytic composites, and are generally peculiar to the environment in which the catalyst is employed. For example, an automotive internal combustion engine is commonly operated over a wide range of speed and load conditions including idling, cruising, accelerating and decelerating, and, therefore, the combustion efficiency of such an engine is varied considerably. The space velocity and temperature of the manifold exhaust gases, as well as the concentration of combustible material therein, will 35 similarly vary over relatively wide limits. Therefore, when applied to the treatment of the noxious exhaust gases from an automotive internal combustion engine, the catalyst must necessarily have the inherent capability of withstanding high temperatures of the order of 1600° F. to as high as about 2000° F., and should possess high 40 activity at substantially lower temperatures. The catalyst should have a relatively low threshold-activation temperature in order that the necessary conversion reactions become self-initiating within a minimum period of time following the startup of the engine at relatively cold conditions. These characteristics have been recognized as essential by the Motor Vehicle Pollution Control Board in 45 setting forth the specifications relating to the efficiency with which the noxious components are eliminated or converted. The catalyst must, therefore, necessarily operate in a satisfactory manner at a temperature which can conceivably vary from about 200° F. to as high as about 50 55 60 65 70 75 80 85 90 95 2000° F., at any given time.

The catalytic composite of the present invention is characterized by the fact that it contains at least one

catalytically active metallic component. As employed in the present specification, as well as in the appended claims, the term "metallic component" is intended to connote those components of the catalyst which are employed for their catalytic activity in converting the noxious material into innocuous components, as distinguished from that portion of the catalyst herein referred to as the refractory inorganic oxide, and which is employed for the purpose of supplying a suitable carrier material, or support, for the "catalytically active metallic components." Although not considered to be a limiting feature of the present invention, it is preferred that the catalytically active metallic component, or components, be composited with a refractory inorganic oxide carrier material which has an apparent bulk density less than about 0.4 gram per cc. Preferred refractory inorganic oxides, for use as the carrier material, possess an apparent bulk density within the range of about 0.15 to about 0.35 gram per cc. The catalytically active metallic components, composited with the refractory inorganic oxide carried material, may be one or more of the following: vanadium, chromium, molybdenum, tungsten, members of the iron-group and platinum-group of the Periodic Table, copper, silver and gold. A particular metal may be used in and of itself, or in combination with any of the foregoing metals. The catalyst of the present invention may comprise a metallic component selected from Groups VA, VIA and VIII of the Periodic Table. Thus, the catalyst to be employed in the treatment of noxious, gaseous combustible waste products, prior to discharging the same into the atmosphere, may comprise the following: platinum, palladium, other noble metals such as iridium, ruthenium and rhodium, iron, cobalt, nickel, copper, vanadium, tungsten, molybdenum, silver, gold, and various mixtures including platinum-iron, platinum-cobalt, platinum-nickel, palladium-iron, palladium-cobalt, palladium-nickel, platinum-palladium, palladium-copper-cobalt, copper-cobalt-nickel-platinum, platinum-palladium-cobalt, etc. It is understood that the catalytic activity, stability, auto-initiating temperature, and other characteristics of the catalyst of the present invention, may vary from catalyst to catalyst. Many of the specific composites discussed herein do not necessarily yield equivalent results when compared with a catalyst comprising one or more different metallic components, or when utilized under varying conditions in different applications. Although the precise manner in which the catalytically active metallic component, such as platinum, is disposed within the carrier material, is not known with absolute certainty, it is believed that the platinum, or other metallic component, enters into a complex combination with the carrier material and other components of the catalyst. Therefore, it is understood that the use of the term "platinum," or "metallic component," for example, connotes platinum, or other metallic components existing within the carrier material in a combined form and/or in the elemental state.

The catalytic composite of the present invention, the method of the preparation of which is hereinafter set forth in greater detail, utilizes a refractory inorganic oxide as the carrier material for the active metallic components hereinbefore set forth. Refractory inorganic oxides possess particular physical characteristics which readily permit adaptation thereof to the rather unique environment encountered in the operation of a motor vehicle, as well as in other commercial applications. One desired physical characteristic, for example, is that extremely high temperatures do not apparently affect the capability of the material to function as desired. The refractory inorganic oxide carrier material, for utilization in the catalyst of the present invention, may be manufactured by any suitable method including separate, successive, coprecipitation means of manufacture when comprising two or more individual inorganic oxides. The car-

rier material may comprise naturally-occurring substances such as clays or earths, and may or may not be activated prior to use by one or more treatments including drying, calcining, steaming, or treatments with various reagents, etc. The catalytic composite of the present invention will preferably make use of an alumina-containing refractory inorganic oxide carrier material; as employed herein, the term "alumina" is intended to include porous aluminum oxide in various states of hydration. In addition to alumina, other refractory inorganic oxides may be employed, either in conjunction with or instead of, the alumina. Other suitable inorganic oxides include silica, boria, thoria, titania, strontia, zirconia, hafnia, and mixtures of two or more. The incorporation of any of the foregoing refractory inorganic oxides, in conjunction with the alumina, is generally dependent upon the desire to add thereto certain physical and/or chemical characteristics required by the particular application for which the catalytic composite is intended. Such other refractory inorganic oxides, for example, silica, will be present within the carrier material in an amount within the range of about 0.5% to about 25.0% by weight thereof, based upon the final weight of the carrier. Intermediate quantities are preferred and will lie within the range of about 1.0% to about 10.0% by weight. The carrier material may take the form of any desired shape such as spheres, pills, extrudates, granules, cakes, briquettes, rings, etc. The preferred form is the sphere, and spheres may be continuously manufactured by the well-known oil-drop method: this method is described in detail in U.S. Patent No. 2,620,314, issued to James Hoekstra. In the interest of simplicity and clarity, the following discussion will be restricted to the use of alumina as the refractory inorganic oxide carrier material. Where desired, halogen may be combined with the alumina and the catalytically active metallic components, and may be added thereto in any suitable manner either before, or after the incorporation of the active metallic components. The addition of the halogen is generally accomplished through the use of an acid such as hydrogen fluoride and/or hydrogen chloride, or volatile salt such as ammonium fluoride and/or ammonium chloride, and the halogen may be combined with the alumina during the preparation of the latter. In still another method of manufacture, the halogen may be composited with a refractory oxide during the impregnation thereof with the catalytically active metallic components. Thus, where the alumina is prepared from an alumina hydrosol having an aluminum to chloride weight ratio of about 1.3, the use of such method permits the incorporation of chloride where the latter is desired as the halogen component.

Regardless of the particular refractory inorganic oxide carrier material employed, the catalytically active metallic components may be added thereto in any suitable, convenient manner. However, in accordance with the present invention, prior to, or during the addition of the metallic component, such as platinum, the preformed inorganic oxide particles, such as alumina, are treated with an organic acid selected from a particular group thereof. In some instances, the organic acid may be combined with the metallic component, for example a water-soluble platinum-containing compound, and the resulting mixture then added to the alumina particles. The selected organic acid may be added to the alumina particles as a separate solution just prior to commingling with the metallic component. For ease in handling the metering, the organic acid is preferably admixed, in the requisite quantity, with the water-soluble compound of the intended catalytically active metallic component, and the resulting impregnating solution combined with the carrier material. With respect to platinum, suitable water-soluble compounds for utilization in the impregnating solution include chloroplatinic acid, chloroplatinous acid, platinous chloride,

platinic chloride, etc. Where the catalytic composite is intended to contain other metallic components, such as those hereinbefore set forth, the composite may be prepared by commingling water-soluble compounds of these components, particularly the nitrates, sulfates, chlorates, chlorides, or carbonates, and immersing the particles of the carrier material therein, followed by heating to form the corresponding oxides of the metallic components.

The organic acid utilized in the method of the present invention, is selected from the group consisting of dibasic acids and derivatives thereof, having the following structural formula:



where:

R is selected from hydrogen, hydroxyl and alkyl groups; R' is selected from hydrogen, alkyl and carboxyl groups; and n is within the range of 0-6.

As hereinafter indicated in a specific example, other organic acids including acetic and tetracetic acids do not suffice to achieve the desired object for which such organic acid is utilized. In accordance with the structural formula given above, suitable organic acids for use in preparing the catalytic composite of the present invention include, but not by way of limitation, oxalic, malonic, succinic, glutaric, adipic, pimelic, suberic, malic, tartaric, citric, 2, methyl succinic, 2,3 di-ethyl succinic, 2,2 di-methyl succinic, mixtures of two or more, etc. The quantity of the dibasic organic acid, or derivative thereof, for example, tartaric acid, to be employed in admixture with the water-soluble compound of the catalytically active metallic component and the carrier material, is based upon the weight of such carrier material. The amount of organic acid employed is within the range of about 0.1% to about 1.5% by weight. An intermediate concentration of the organic acid and/or its derivative is preferred, and is within the range of from about 0.13% to about 0.70% by weight, based upon the weight of the carrier material. Through the utilization of the method of the present invention which principally comprises treating the carrier material with a particular quantity of a particular organic acid, the use of lesser quantities of the active metallic components to achieve the desired end result is permitted.

The quantity of the catalytically active metallic components is based upon the volume of the carrier material to be combined therewith, and is calculated on the basis of the elemental metal, notwithstanding that the metallic component may exist in some combined complex form, or in the elemental state. Thus, with respect to platinum-group metals, the platinum will be present in an amount of from about 0.05 to about 1.0 troy ounce per cubic foot of carrier material. The preferred range of the concentration of the platinum component, dictated by economic considerations, is from about 0.15 to about 0.60 troy ounce per cubic foot of carrier material. The other metallic components, either in conjunction with, or instead of the platinum component, will be present in an amount of from about 0.01 to about 2.0 troy ounces per cubic foot of carrier material employed.

The organic acid may be employed as a mixture of two or more, and may be diluted with any suitable non-alkaline solubilizing substances such as water, alcohol, acetone, etc. Of the organic acids above set forth, citric, oxalic, and tartaric acids are the preferred organic acids to be employed in the method of the present invention, citric acid being particularly preferred. The organic acid may be admixed with the water-soluble compound of the catalytically active metallic component, or components, or mixed with the alumina prior to the addition of the metallic component thereto. In any case, it is an essen-

tial feature of the present invention that the metallic component be not combined with the alumina prior to the addition of the organic acid. Another essential feature of the present invention is that the commingling of the refractory inorganic oxide, the catalytically active metallic component and the organic acid be accomplished in the absence of substances and reagents of an alkaline nature, particularly including ammonia and other nitrogenous compounds, alkali metal compounds, etc. It has further been found that the catalytic composite is adversely affected when contacted with a nitrogen-containing gas during the final high-temperature stages of the manufacture thereof.

In describing the method of manufacturing the catalytic composite encompassed by the present invention, it is understood that the same is not considered to be unduly limited to the particular catalytic composite described. The catalyst is prepared by initially forming alumina spheres,  $\frac{1}{16}$ -inch to about  $\frac{1}{8}$ -inch in diameter, from an aluminum chloride hydrosol having an aluminum chloride weight ratio of about 1.25. The alumina spheres are continuously prepared by passing droplets of the hydrosol into an oil bath maintained at an elevated temperature, retaining the droplets within the oil until the same set into hydrogel spheroids. The spheroids are dried at a temperature of from about 200° F. to about 800° F., and thereafter subjected to a calcining treatment at a temperature of from about 800° F. to about 1200° F. An impregnating solution of chloroplatinic acid, having the concentration of 0.0628 gram of platinum per milliliter, is prepared by diluting 3.0 milliliters to about 500 milliliters with water. When utilized with about 150 grams of the alumina spheres, having an apparent bulk density of about 0.29 gram per cc., this concentration of the chloroplatinic acid solution will yield a final composite having about 0.32 troy ounce of platinum per cubic foot of the spherical alumina carrier material. The chloroplatinic acid solution is commingled with about 0.52 gram of citric acid, or 0.35% by weight based upon the weight of the alumina spheres. The resulting mixture of citric acid, chloroplatinic acid and alumina spheres is evaporated to dryness in a rotating dryer at a temperature of about 210° F. When the alumina spheres appear visually dry, usually in about 2 to about 8 hours, the impregnated spheres are subjected to a reducing treatment, preferably in an atmosphere of hydrogen, while increasing the temperature to a level within the range of about 900° F. to about 1800° F., maintaining the elevated temperature for about 2 hours. Contrary to present-day methods of manufacturing catalytic composites, the catalyst of the present invention is not subjected to an oxidation treatment at elevated temperature, or to high-temperature calcination in an atmosphere of air. A high-temperature oxidation treatment tends to destroy both the initial activity, and more particularly the stability of the catalytic composite to effect the removal and/or conversion of the noxious components in the combustible gaseous waste products. Furthermore, oxidation in air will cause the catalytic composite to come in contact with nitrogen at an elevated temperature, and, as hereinafter indicated, such treatment tends to destroy the stability of the catalytic composite.

From the foregoing description of the present invention, it will be noted that the inorganic oxide carrier material is combined with the catalytically active metallic component in the presence of a particular quantity of an organic acid selected from the group consisting of dibasic organic acids and derivatives thereof, having the following structural formula:



where:

R is selected from hydrogen, hydroxyl and alkyl groups; R' is selected from hydrogen, alkyl and carboxyl groups; and n is within the range of 0 to 6.

The concentration of the organic acid is from about 0.1% to about 1.5%, and is based upon the weight of the carrier material to be impregnated with the active metallic component. It is recognized that the prior art teaches broadly the "activation" of refractory inorganic oxides through the utilization of various reagents including organic acids. Such "activation" is, however, immediately followed by a high-temperature calcination treatment prior to the incorporation of the catalytically active metallic components. However, the particular concentration of the organic acid, as utilized in the method of the present invention, and in the manner set forth, results in a catalytic composite having a physical structure heretofore not obtained. This phenomenon is more clearly described and illustrated in the accompanying FIGURES 1, 2, 3 and 4. These figures illustrate the cross section of an alumina spherical particle, taken through the center thereof, which particle contains a platinum component as the catalytically active metallic component. With reference now to the figures, FIGURE 1 illustrates an alumina-platinum composite prepared in the absence of the organic acid, or with an organic acid in a concentration less than about 0.10% by weight based upon the weight of alumina. In the figure, numeral 1 denotes the exterior surface of the entire sphere, numeral 2 denotes a continuous finite layer of the platinum component and numeral 3 refers to the porous alumina core, noted to be virtually free from the platinum component. It will be further noted, upon reference to FIGURE 1, that the absence of the organic acid, or the use of too little organic acid during the impregnation of the sphere, has produced a catalytic particle in which virtually the entire quantity of the catalytically active metallic component resides on the surface thereof.

With reference to FIGURE 2, illustrating the cross-section of an alumina sphere impregnated with a platinum component and a dibasic acid, and/or derivative thereof, from the group of acids hereinbefore defined, in accordance with the method of the present invention, numeral 1' connotes the exterior surface of the entire sphere, 2' refers to the totally imbedded continuous layer of the platinum component, 3' indicates the inner core of alumina (virtually free from the platinum component), and numeral 4 indicates an outer band of alumina also virtually free from the platinum component. It is noted that the use of the present invention has produced a catalytic particle in which the catalytically active metallic component is imbedded as a layer within the refractory inorganic oxide, and is disposed a finite distance from the exterior surface and a finite distance from the center thereof.

With reference to FIGURE 3, 1" denotes the entire spherical particle, 2" a virtually solid inner core of the platinum component and 3" indicates a wide outer band of substantially pure alumina. The catalytic particle illustrated in FIGURE 3 results when the organic acid is employed in a concentration greater than about 1.5% by weight, based upon the weight of the alumina. Upon reference to FIGURE 4, 1"" denotes the entire spherical particle and 2"" denotes the alumina interior in which the platinum component is quite thoroughly and evenly distributed. The catalytic particle having the structural character illustrated in FIGURE 4, results when the organic acid is employed in the presence of ammonia or other alkalinous-acting material, notwithstanding that the organic acid concentration may lie within the range of from about 0.1% to about 1.5% by weight.

In addition to the aliphatic, organic dibasic acids, and derivatives thereof hereinabove described, aromatic or-

ganic acids containing a hydroxyl group adjacent to the carboxylic group have been found which when employed in accordance with the method of the present invention, produce a catalytic particle having the structure shown in FIGURE 2. For example, salicylic acid, when utilized in an amount within the range of about 0.1% to about 1.5% produced a platinum-containing catalytic particle in which the totally imbedded layer of the platinum component was clearly visible to the naked eye. Derivatives of such aromatic, organic acids, including gamma resorcyclic acid, and others having a hydroxyl group adjacent the carboxylic group, also result in such a physical structure.

It is readily ascertained that the use of the method of the present invention has produced a catalytic particle having a novel physical structure in which the active metallic component is completely imbedded as a layer within the particle, and is disposed a finite distance from the center and exterior surface of the particle. As hereinbefore indicated and set forth, in specific examples, the catalytic particle of the character represented in FIGURE 2 possesses the requisite stability of a catalytic composite intended to serve the function of eliminating noxious components from gaseous combustible waste products, and particularly for converting the hydrocarbonaceous gaseous waste products emanating from the exhaust of an internal combustion engine. Catalytic particles having physical structures illustrated by FIGURES 1, 3 and 4, either have a high initial activity and virtually no stability, or substantially no conversion activity and a high degree of stability. FIGURES 1, 2, 3 and 4 were made from cross-sectional photographs of spherical alumina-platinum composites prepared in conjunction with the specific examples hereinafter set forth. The impregnated platinum component was made more visible and contrasting through the use of stannous chloride. Although only spherically shaped particles have been illustrated, it is understood that the method of the present invention is adaptable for utilization with inorganic oxide particles of any desired shape. For example, in the case of an alumina particle having the shape of the well-known Raschig ring, a horizontal cross section would show the hollow center, characteristic of the Raschig ring, a band of alumina substantially free from the platinum component, a continuous layer of the platinum component which has been impregnated completely within the alumina, and lastly, an outermost band of alumina substantially free from the platinum component.

The following examples are given for the purpose of illustrating clearly the method of manufacturing the catalytic composite encompassed by the present invention. It is understood that the present invention is not to be unduly limited, beyond the scope and spirit of the appended claims, by the conditions, reagents, concentrations, or catalytic composites employed within the examples. When considered in conjunction with the accompanying FIGURES 5 through 11, the data presented within the examples will indicate the benefits to be afforded through the utilization of the present invention, which invention produces a catalytic composite having the physical structure illustrated in accompanying FIGURE 2. It will be readily ascertained that the catalytic composite offers particular advantages in a process for the elimination of the products of incomplete combustion from the hydrocarbonaceous exhaust gases emanating from an internal combustion engine, by which method such exhaust gases become innocuous upon being discharged into the atmosphere.

#### Example I

The catalysts employed in this example were prepared by initially forming alumina spherical particles of  $\frac{1}{8}$ -inch diameter and having an apparent bulk density of about 0.29 gram per cc. The two catalysts were prepared in such a manner that the concentrations of cat-

alytically active metallic component were identical, and the entire manufacturing process would be the same with but one exception; that is, one catalyst was prepared by effecting the impregnation in the presences of citric acid, in accordance with the method of the present invention. The  $\frac{1}{8}$ -inch alumina spheres were divided in two separate portions, each being impregnated with a sufficient quantity of chloroplatinic acid (having a concentration of 0.0628 gram of platinum per milliliter) to yield a catalyst containing 0.47 troy ounce of platinum, calculated as the element thereof, per cubic foot of alumina. For each 150 grams of the alumina spheres, the required quantity of chloroplatinic acid was diluted to 500 milliliters with water. Prior to being impregnated, the impregnating solution for one catalyst portion was admixed with 0.22% by weight of citric acid, based upon the total quantity of alumina particles. Both catalyst portions were individually and separately evaporated to dryness in a rotating dryer at a temperature of about 210° F. While increasing the temperature to a level of about 1000° F., the catalyst portions were subjected to an atmosphere of hydrogen; after reaching a temperature level of 1000° F., the hydrogen treatment was continued at that temperature for a period of 2 hours. The catalyst portions were allowed to cool prior to being exposed to the atmosphere.

The two catalyst portions were then subjected to chassis dynamometer road testing in accordance with the 7-mode cycle set forth in the Vehicular Exhaust Emission specification approved by the Motor Vehicle Pollution Control Board of the State of California. The Vehicular Exhaust Emission specifications herein referred to are those which were approved on May 19, 1961. Aside from the specific limitations placed upon the method of testing, which limitations were strictly adhered to during the chassis dynamometer testing, the specification includes a maximum tolerable limit with respect to the concentration of hydrocarbons and carbon monoxide within the exhaust gases of the internal combustion engine. The maximum tolerable limit on hydrocarbon concentration is 275 p.p.m., the tolerable concentration of carbon monoxide being less than 1.5%. With reference now to FIGURE 5, dotted line 1 indicates the tolerable limit on hydrocarbons of 275 p.p.m. Line 2, drawn through the circles, indicates the results obtained through the use of catalyst prepared in the absence of the citric acid; it is noted that this catalyst exceeded 275 p.p.m. of hydrocarbons in the exhaust gas at approximately 2000 miles. Line 3 illustrates the results obtained through the use of the catalyst of the present invention, during the preparation of which citric acid was employed in the impregnating solution. It is noted that the hydrocarbon concentration in the exhaust gases did not exceed 275 p.p.m. for the 8000 miles illustrated, and, in fact, appears to indicate a slightly downward trend. One of the more important aspects of the data as presented in FIGURE 5 is the apparently greater degree of stability of the catalyst prepared by the method incorporating the use of citric acid.

Similarly, FIGURE 6 illustrates the comparison of the two catalytic composites with respect to the concentration of carbon monoxide in the exhaust gases. Line 1 represents the results of the catalyst prepared in the absence of citric acid, while line 2 illustrates the results obtained through the use of the catalyst of the present invention. Although the carbon monoxide concentration for both catalysts is below the 1.5% specified limit, it is readily ascertained that the catalyst of the present invention possesses greater stability and will function acceptably, with respect to carbon monoxide concentration, for a period of time much longer than the catalyst prepared in the absence of the citric acid.

The data employed in the illustrations embodied by FIGURES 5 and 6 are given in the following table, in which "A" designates the catalyst prepared in the ab-

sence of citric acid; B designates the catalyst prepared in accordance with the present invention:

TABLE—MVPB<sup>1</sup> SEVEN-MODE CYCLE ROAD TESTING

| Catalyst Life, Miles | Hydrocarbons, p.p.m. |       | Carbon Monoxide, percent |       |
|----------------------|----------------------|-------|--------------------------|-------|
|                      | A                    | B     | A                        | B     |
| 10 0.....            | 165                  | 166   | 0.26                     | 0.27  |
| 501.....             | 174                  | 185   | 0.34                     | 0.23  |
| 1,013.....           | 242                  | 188   | 0.38                     | 0.25  |
| 1,521.....           | 289                  | ..... | 0.43                     | ..... |
| 2,007.....           | 336                  | 215   | 0.45                     | 0.29  |
| 3,085.....           | 323                  | 215   | 0.43                     | 0.38  |
| 4,137.....           | 331                  | 268   | 0.48                     | 0.30  |
| 6,000.....           | 387                  | 250   | 0.63                     | 0.40  |
| 8,031.....           | 229                  | ..... | 0.48                     | ..... |

<sup>1</sup> Motor Vehicle Pollution Control Board.

The 7-mode road testing cycle prescribed by the Vehicular Exhaust Emission specifications is a chassis dynamometer test procedure. A single cycle covers a total period of time of 137 seconds, the seven modes being as follows: (1), idling; (2), acceleration to 30 miles per hour; (3), cruise at 30 miles per hour; (4), deceleration to 15 miles per hour; (5), cruising at 15 miles per hour; (6), acceleration to 50 miles per hour; and (7), deceleration to idle. From a cold start-up, the specifications require an operation of 7 to 8 cycles, the first four considered as the warm-up period which includes a cold start, the 7th or 8th cycle being considered the hot cycle. The maximum limitations placed upon the hydrocarbon concentration, p.p.m., and the carbon monoxide, in percent, is specified as being the sum of 45% of the average of four warm-up cycles and 55% of a single hot cycle. The data presented in the foregoing table, and employed in FIGURES 5 and 6, were obtained in accordance with the foregoing Vehicular Exhaust Emission specifications.

The following examples are those which were employed in obtaining the data illustrated in the accompanying FIGURES 7, 8, 9, 10 and 11, and utilized a specific catalyst evaluation test procedure designed to determine the catalytic stability with respect to automotive exhaust conversion. The various catalytic composites are evaluated by a test procedure which simulates actual driving conditions. The test procedure involves the utilization of a standard dynamometer, by which an 8-cylinder internal combustion engine is loaded, or driven, by a motor-generator. Approximately 440 cc. of each of the catalyst portions are individually evaluated by being placed within a cylindrical vessel, or convertor, having an inside diameter of about 4 inches, the entire apparatus being serially connected into the engine exhaust line. The catalyst sample is disposed within the convertor on a supporting screen to a bed height of about 2 to about 3 inches. A second screen is placed above the catalyst bed for the purpose of separating the catalyst from the  $\frac{1}{4}$ -inch ceramic balls employed to facilitate the even distribution of the exhaust gases flowing downwardly through the apparatus. Four such catalyst-loaded convertors are utilized in a given test period; this practice permits the simultaneous testing of different catalysts, and provides an excellent basis for making a comparative study of the results.

Combustion air is pressured into the convertor inlet, the flow rate being adjusted such that the average temperature of the catalyst bed is maintained at a level within the range of about 800° F. to about 1700° F. It is preferred that the flow rate of combustion air be held constant at about six pounds per hour, such that the catalyst bed average temperature is maintained at a level of about 950° F. The fuel employed in the test procedure is a blend of catalytically reformed gasoline (40.0%), catalytically cracked gasoline (40.0%) and alkylate (20.0%), and contains 3.0 milliliters of tetraethyl lead per gallon. Since the concentration of unburned hydrocarbons, and other noxious products, within the exhaust

gases, as well as the throughput thereof, varies in accordance with the physical status of the engine, whether idling, accelerating, cruising or decelerating, the test procedure still further approximates actual road conditions by providing for a constant load throughout only a portion of the entire test period. Samples of the convertor inlet and outlet gases are taken at various intervals during the test procedure, there being a constant analysis for the concentration of carbon monoxide. The samples are analyzed for hydrocarbons by a flame-ionization detector. The term "hydrocarbon," as utilized in reporting the results of the analyses performed on the effluent gases from the catalytic convertor, connotes all hydrocarbons whether saturated, unsaturated, or partially oxidized as hereinbefore set forth. The carbon monoxide concentration within the exhaust gases is determined by an accurate infra-red detector. The internal combustion engine is operated in a particular cycle to simulate idling, accelerating, cruising and decelerating as experienced under actual road conditions. During the entire test procedure, which covers a period of about 40 hours, about 300 gallons of the aforementioned fuel is employed. The 40-hour test period is divided into eight five-hour cycles; each five-hour cycle consists of a four and one-half hour cruise at a constant 2500 r.p.m. and 41 B.H.P., and a one-half hour cycle consisting of a series of 15 two-minute cycles comprising idling at 750 r.p.m., accelerating to cruise at 2000 r.p.m., and a deceleration to idling at 750 r.p.m.

An inherent result of the small volume of catalyst employed in the test evaluation procedure is that the space velocity of the exhaust gases coming into contact with the catalyst is considerably higher than would usually be encountered under actual driving conditions. Accordingly, the percentage conversion obtained during actual use in automotive exhaust gas convertors would be considerably higher. The data obtained from the 40-hour test procedure is plotted on semi-logarithmic coordinates and results in a curve from which the following equation is derived:

$$C = Ae^{-t/k}$$

In the equation,  $k$  equals the reciprocal of the slope,  $A$  equals the percent initial conversion obtained by extrapolation,  $C$  equals the percent conversion in time ( $t$ ), and  $t$  equals the time in hours. The above equation is employed in computing the " $k$ " stability factors for the individual catalytic composites. A decrease in the slope of the curve resulting from the data obtained, or conversely, an increase in " $k$ " value, indicates a catalyst possessing a greater degree of stability when converting the hydrocarbonaceous combustion products of an internal combustion engine. In those instances where the " $k$ " stability factor is positive, indicating a positive slope, the stability of the catalyst being evaluated may be said to increase with time.

The foregoing described test procedure is employed as a primary evaluation of the catalysts intended to be subjected to the 7-mode cycle operation described in conjunction with the foregoing Example I. The importance of this primary evaluation resides in the " $k$ " stability factor of the catalytic composite being tested. That is, although a wide variety of catalytic composites possess a relative high initial activity, the stability of such catalysts is such that the maximum tolerable limits imposed upon the hydrocarbon and carbon monoxide concentrations are reached in a relatively short period of time.

#### Example II

This example is presented for the purpose of illustrating the adverse effects upon the catalytic composite which has been subjected to high-temperature treatment in an atmosphere of nitrogen. These catalysts were prepared utilizing the alumina spheres and chloroplatinic acid solution described in Example I; however, the impregnation

of the spheres with the chloroplatinic acid was not conducted in the presence of an organic acid selected from the group hereinbefore set forth. The chloroplatinic acid solution was employed in an amount such that the final catalytic composite contained 0.19 troy ounce of platinum, calculated as the element, per cubic foot of alumina. Following the drying of the impregnated alumina spheres, at a temperature of about 210° F., the temperature was increased in the first instance to a level of 1000° F., in the presence of nitrogen, and maintained at this level for a period of 2 hours. In a second instance, the catalyst temperature was increased to a level of 1500° F., in the presence of nitrogen, again remaining at this level for a period of 2 hours. The results of the automotive exhaust conversion test procedure, with respect to the two nitrogen-treated catalysts, are presented in FIGURE 7.

With reference to FIGURE 7, lines 1 and 2 represent the stability curves of the catalyst treated at 1000° F., for the conversion of carbon monoxide and hydrocarbons respectively. The " $k$ " stability factors, derived from lines 1 and 2 by means of the previously indicated equation are 79.5 with respect to carbon monoxide and 68.2 with respect to the concentration of hydrocarbons. Lines 3 and 4 represent the results of the evaluation of the catalyst which had been nitrogen-treated at a temperature of 1500° F. The " $k$ " stability factors were found to be 61.4 for carbon monoxide and 49.3 with respect to the concentration of hydrocarbons. A standard reference catalytic composite, containing 0.19 troy ounce of platinum per cubic foot of alumina, prepared in the absence of an organic acid, however, with a high-temperature treatment in the presence of hydrogen rather than nitrogen, indicates a " $k$ " stability factor of about 90 to 120 with respect to the concentration of hydrocarbons and a stability factor of about 110 to about 150 with respect to the concentration of carbon monoxide. Upon comparing the " $k$ " stability factors, it is readily noted that the high-temperature treatment in an atmosphere of nitrogen has adversely effected the platinum-containing catalyst of the type commonly manufactured by present-day operations.

Also illustrated in FIGURE 7 are the results of the evaluation test with respect to a catalytic composite of alumina and platinum prepared by the method commonly referred to as "co-precipitation." The co-precipitation method of manufacturing allegedly results in a catalytic composite in which the catalytically active metallic component, in this case platinum, is thoroughly and evenly distributed throughout the carrier material. A cross section of a catalyst of this nature would have the appearance of the catalytic particle illustrated in FIGURE 4. The results of the evaluation test procedure on the co-precipitated catalyst indicated a stability factor of 59.4 with respect to carbon monoxide and 36.1 with respect to the concentration of hydrocarbons. When compared to the " $k$ " stability factors of the standard catalyst, it is readily ascertained that the co-precipitated catalyst is not readily adaptable to the process of eliminating the noxious components from automotive exhaust gases, notwithstanding that such co-precipitated catalysts, having the physical structure as indicated in FIGURE 4, are considered to be highly advantageous when employed in processes specifically designed for the catalytic reforming of various hydrocarbon mixtures to produce high quality motor fuel.

#### Example III

The data obtained in this example is illustrated in the accompanying FIGURE 8. The first catalyst was prepared in accordance with the method described in reference to Example I, utilizing sufficient chloroplatinic acid to yield a final composite containing 0.19 troy ounce of platinum per cubic foot. During the impregnation of the alumina spherical particles with the chloroplatinic acid, 1.05 grams of acetic acid were added for each 150 grams of alumina spheres, or acetic acid in an amount of about 0.70% by weight. The results of the catalyst evaluation

test, with respect to the acetic acid-treated catalyst are indicated in FIGURE 8 by stability lines 1 and 2, representing "k" stability factors of 90.7 with respect to the quantity of carbon monoxide, and 73.4 with respect to the concentration of hydrocarbons, respectively. The standard reference catalyst, tested simultaneously with the acetic acid-treated catalyst, but in a separate convertor as stated in the foregoing description of the test procedure, indicated stability factors of 118.7 and 163.9 respectively. The effect of the use of acetic acid, resulting in a catalytic particle having the physical structure illustrated by FIGURE 4, has been to decrease the degree of stability of the catalytic composite as indicated by a change in the hydrocarbon stability factor from 118.7 to 73.4; the stability factor for carbon monoxide decreasing from 163.9 to 90.7. Thus, the utilization of acetic acid, notwithstanding its similarity to oxalic, citric and/or tartaric acids, is seen to be non-applicable in preparing a catalyst for the conversion and/or removal of noxious components from automotive exhaust gases.

A second catalyst was prepared by the method set forth in Example I, utilizing sufficient chloroplatinic acid to result in a catalyst containing 0.32 troy ounce of platinum per cubic foot, impregnated in the presence of 1.08% by weight of citric acid, based upon 170 grams of the alumina spherical particles. The results obtained through the utilization of the citric acid treated catalyst are indicated by lines 3 and 4 in FIGURE 8, illustrating the stability curves for carbon monoxide and hydrocarbons respectively. It should be immediately noted that line 3 possesses a positive slope, the "k" stability factor being calculated as 2731.5+, compared to 116.3 for the standard reference catalyst. The "k" stability factor with respect to hydrocarbon concentration was found to be 115.5, indicated in FIGURE 8 by line 4, compared to 68.5 for the standard. The importance of the data illustrated in FIGURE 8 resides in the fact that the stability curves, lines 3 and 4, for the citric acid-treated catalyst are virtually horizontal, indicating a catalytic composite possessed with an unusually high degree of stability when employed in the conversion of carbon monoxide and the hydrocarbonaceous material contained within the exhaust gases of an automotive internal combustion engine.

#### Example IV

This example is presented to show the results obtained from the evaluation test procedure comparing the standard catalyst and a catalyst prepared through the use of 0.35% by weight of citric acid, based upon the quantity of alumina, during the impregnation of the latter with sufficient chloroplatinic acid to result in a catalyst containing 0.32 troy ounce of platinum per cubic foot. The acid-treated catalyst and the standard catalyst were simultaneously subjected to the catalyst evaluation test procedure, however, having been placed in individual convertors through which the engine exhaust gases were passed. The results are graphically illustrated in accompanying FIGURE 9, lines 1 and 2 indicating the stability curves of the standard reference catalyst, lines 3 and 4 indicating the stability curves of the citric acid-treated catalyst. The citric acid-treated catalyst indicated a "k" stability factor of 208.5 with respect to the quantity of hydrocarbons, the standard reference catalyst indicating a "k" stability factor of 90.8; the stability factor with respect to carbon monoxide, resulting from the use of the citric acid-treated catalyst indicated a slightly positive slope (line 3), calculated as 12120.1+, whereas the carbon monoxide "k" stability factor for the standard reference catalyst was 125.5.

In order to illustrate the detrimental effects exhibited when the catalyst is prepared in the presence of alkalinous material, such as ammonia, a catalyst was prepared in accordance with the method of the present invention utilizing 0.35% by weight of citric acid, based upon the weight of alumina particles, during the impregnation of

the chloroplatinic acid solution to yield a catalyst containing 0.32 troy ounce of platinum per cubic foot. The "k" stability factor with respect to the concentration of hydrocarbons was 126.5, a significant decrease from 208.5 as hereinabove indicated; the carbon monoxide "k" stability factor was 214.7, substantially less than the positive slope indicated by the catalyst prepared by the method excluding alkalinous material. The ammonia-treated catalyst was prepared by including 181 milligrams of ammonia in the citric acid-chloroplatinic acid impregnating solution, resulting in a pH thereof of about 7.0.

This particular example illustrates clearly the benefits afforded through the utilization of the present invention, particularly with respect to the use of an organic acid in relatively minor concentration; the present invention unquestionably produces a highly stable catalytic composite. The example illustrates the detrimental effects of the presence of ammonia and/or other alkalinous material during the impregnation of the carrier material with the catalytically active metallic component.

#### Example V

Three different catalytic composites were prepared in obtaining the data presented in this example; reference is made, in this example, to accompanying FIGURE 10 which illustrates the results of the 40-hour catalyst evaluation procedure. The first catalyst was prepared to contain 0.32 troy ounce of platinum per cubic foot, which had been impregnated within the alumina spherical particles in the absence of an organic acid. However, following the high-temperature reduction treatment in hydrogen, the catalytic composite was cooled and treated with 1.46 grams of citric acid per 150 grams of alumina, or 0.97% by weight of citric acid. The results of the 40-hour test procedure are indicated as lines 1 and 2 in FIGURE 10; the stability factors obtained with respect to this catalyst were 142.9 in regard to the carbon monoxide, and 104.6 with respect to the hydrocarbon concentration. The standard reference catalyst, tested simultaneously in a separate convertor, indicated a "k" stability factor of 125.5 and 90.8 respectively. There would appear to be a slight improvement over the standard catalyst in treating such a catalyst with the organic acid following a high-temperature treatment. However, it will be noted that the improvement in "k" stability factors is quite small, especially when compared to the second catalyst, the results of which are represented by lines 3 and 4 in FIGURE 10. The second catalyst was prepared to contain 0.32 troy ounce of platinum per cubic foot, which platinum was impregnated within the alumina in the presence of 0.35% by weight of citric acid, based upon the quantity of alumina. This catalyst was tested simultaneously with the two above-described catalytic composites, and indicated a "k" stability factor for hydrocarbons of 208.5; it will be noted, upon reference to FIGURE 10, that the "k" stability factor for carbon monoxide was positive, the slope of line 3 indicating a slight rise.

The third catalyst illustrated in FIGURE 10, by lines 5 and 6, was prepared to contain 0.32 troy ounce of platinum impregnated in the presence of 3.47% by weight of citric, which amount is in excess of the upper limit imposed thereupon. The use of such an excess of organic acid produces a catalytic particle having the physical structure indicated by FIGURE 3, in which virtually all of the metallic component is forced into the center of the spherical particle. The "k" stability factors of this catalyst were substantially less than the standard reference catalyst, being 36.8 with respect to the hydrocarbon concentration and 48.7 in regard to carbon monoxide. The three catalysts represented by the data presented in FIGURE 10, were simultaneously tested in accordance with the catalyst evaluation test procedure. Therefore, a direct comparison of the three methods of catalyst manufacture may be made upon reference to FIGURE 10. It is readily ascertained that the utilization of an excess

of the organic acid, or the use of the organic acid after the metallic component has been combined with the inorganic oxide particle, does not serve to attain the desired object of the present invention. This is very clearly illustrated in FIGURE 10, through the use of lines 1, 2, 5 and 6.

*Example VI*

In this example, the results of which are illustrated in FIGURE 11, a direct comparison was made between the standard reference catalyst and a catalyst containing 0.51 troy ounce of platinum impregnated in the presence of 0.53% by weight of citric acid, based upon the weight of the alumina particles. The catalytic composites were simultaneously, but separately, subjected to the catalyst test evaluation procedure to determine the slope of the stability curve. These curves are indicated in FIGURE 11 in the following manner: line 1 is the carbon monoxide stability curve of the standard reference catalyst, line 2 represents the hydrocarbon stability curve; lines 3 and 4 represent the carbon monoxide and hydrocarbon stability curves respectively of the citric acid-treated catalyst. It is immediately noted that lines 3 and 4 both are characterized by having a positive slope, indicating an increase in stability with time. The citric acid-treated catalyst had a hydrocarbon "k" stability factor of 475.6+ compared to 125.5 for the standard reference catalyst, the carbon monoxide "k" stability factor was 289.3+ compared to 160.9 for the reference catalyst.

Following the first 40-hour test procedure, the catalytic composites were removed from the individual convertors for the purpose of inspecting the same. It was decided to extend the duration of the test procedure, with respect to these two catalysts, by re-loading the convertors, and subjecting the catalysts to a second 40-hour test procedure. The stability curves for the second 40-hour evaluation test are indicated by lines 1A and 2A, for the standard reference catalyst and lines 3A and 4A for the citric acid-treated catalyst. The break in these lines at the 40-hour duration results from the fact that the catalysts had been removed from the individual convertors to enable the visual inspection thereof. The importance of the data presented in FIGURE 11 resides in the fact that the extended stability curves from 40 to 80 hours indicates substantial continued improvement over the standard catalyst. It is of further interest to note that the improvement over the standard catalyst is greater at 80 hours than it was at the termination of the first 40-hour test procedure.

*Example VII*

A catalyst was prepared to contain 0.32 troy ounce of platinum, impregnated within the alumina carrier material in the presence of 1.4 grams of tartaric acid per 150 grams of the alumina, or 0.93% by weight of tartaric acid. As illustrated in accompanying FIGURE 12, an extended duration stability test was made on this particular catalytic composite. In FIGURE 12, line 1 indicates the stability curve with respect to carbon monoxide, line 2 the stability curve with respect to the conversion of hydrocarbons, line 1A the continued stability curve with respect to carbon monoxide and 2A the continued stability curve with respect to the conversion of hydrocarbons. With respect to lines 1 and 2, the "k" stability factors for the tartaric acid-treated catalyst were 860.7+ and 242.1 respectively; the "k" stability factors for the standard reference catalytic composite were 189.5 and 110.7 respectively. This substantial improvement in stability was similarly pronounced during the extended period of 40 to 80 hours.

The foregoing examples present data which clearly indicate the benefits afforded through the use of a catalytic composite having the physical structure encompassed by the present invention, and prepared in accordance therewith. The utilization of a particular concentration of an organic acid, during the impregnation of the refractory

5

inorganic oxide carrier material with the catalytically active metallic component, results in a catalytic composite having an unusually high and totally unexpected degree of stability with respect to the conversion or elimination of the noxious components contained within the exhaust gases from an automotive internal combustion engine, such that these exhaust gases may be discharged into the atmosphere with significantly less noxious characteristics.

I claim as my invention:

1. A method for conversion by oxidation of noxious, gaseous combustible waste products to be discharged into the atmosphere which comprises adding an oxygen-containing gas thereto and contacting the resulting gas mixture, at conversion conditions, with a platinum group metal-alumina catalyst prepared by commingling alumina with a platinum-group metal component and from about 0.1% to about 1.5% by weight, based upon the weight of said alumina, of an organic acid selected from the group consisting of dibasic acids and derivatives thereof, having the following structural formula:

25



where:

- 30 R is selected from hydrogen, hydroxyl and alkyl groups;
- R' is selected from hydrogen, alkyl and carboxyl groups; and
- n is within the range of 0 to 6;

and thereafter heating the resulting catalytic mixture in an atmosphere of hydrogen to an elevated temperature.

- 40 2. A method for eliminating by oxidation the hydrocarbons from gases containing the same which comprises adding an oxygen-containing gas thereto and contacting the resulting gas mixture, at conversion conditions, with a catalytic composite of alumina and a platinum component, said catalytic composite being prepared by initially commingling said alumina with a platinum-containing compound and from about 0.13% to about 0.70% by weight, based upon the weight of said alumina, of an organic acid selected from the group consisting of dibasic acids and derivatives thereof, having the following structural formula:

50



where:

- 55 R is selected from hydrogen, hydroxyl and alkyl groups;
- R' is selected from hydrogen, alkyl and carboxyl groups; and
- n is within the range of 0 to 6;

and thereafter heating the resulting catalytic mixture in an atmosphere of hydrogen to a temperature of about 900°-1800° F.

- 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 92

acids and derivatives thereof having the following structural formula:



where:

R is selected from hydrogen, hydroxyl and alkyl groups;

R' is selected from hydrogen, alkyl and carboxyl groups; and

n is within the range of 0 to 6;

and thereafter heating the resulting catalytic mixture in an atmosphere of hydrogen to a temperature of about 900°-1800° F.

4. A method for eliminating by oxidation by products of incomplete combustion from the hydrocarbonaceous exhaust gases emanating from an internal combustion engine which comprises adding an oxygen-containing gas to said exhaust gases, contacting the resulting gas mixture, at conversion conditions, with a catalytic composite of alumina and a platinum component imbedded as a layer within said alumina and disposed a finite distance below the surface of said alumina and a finite distance from the center thereof; said catalytic composite having been prepared by initially commingling said alumina with a platinum-containing compound and from about 0.13% to about 0.70% by weight, based upon the weight of said

alumina, of an organic acid selected from the group consisting of dibasic acids and derivatives thereof, having the following structural formula:



where:

R is selected from hydrogen, hydroxyl and alkyl groups;

R' is selected from hydrogen, alkyl and carboxyl groups; and

n is within the range of 0 to 6;

drying the resulting catalytic mixture at a temperature within the range of about 100°-250° F., and thereafter heating the catalytic mixture in an atmosphere of hydrogen to a temperature of about 900°-1800° F.

References Cited by the Examiner

UNITED STATES PATENTS

2,927,088 3/1960 Michalko et al. 252—466  
3,133,029 5/1964 Hoekstra 23—2 X

25 OSCAR R. VERTIZ, Primary Examiner.

MAURICE A. BRINDISI, BENJAMIN HENKIN,  
Examiners.

E. C. THOMAS, Assistant Examiner.